



US007683224B2

(12) **United States Patent**  
**Connor**

(10) **Patent No.:** **US 7,683,224 B2**  
(45) **Date of Patent:** **Mar. 23, 2010**

(54) **FUEL FOR JET, GAS TURBINE, ROCKET  
AND DIESEL ENGINES**

(75) Inventor: **Daniel Stedman Connor**, Cincinnati, OH (US)

(73) Assignee: **The Procter & Gamble Company**, Cincinnati, OH (US)

(\*) Notice: Subject to any disclaimer, the term of this patent is extended or adjusted under 35 U.S.C. 154(b) by 845 days.

(21) Appl. No.: **10/902,729**

(22) Filed: **Jul. 29, 2004**

(65) **Prior Publication Data**

US 2005/0027148 A1 Feb. 3, 2005

**Related U.S. Application Data**

(60) Provisional application No. 60/491,721, filed on Aug. 1, 2003.

(51) **Int. Cl.**  
**C10L 1/16** (2006.01)  
**C07C 9/00** (2006.01)

(52) **U.S. Cl.** ..... **585/14; 208/15**

(58) **Field of Classification Search** ..... **585/15,  
585/14; 208/15**

See application file for complete search history.

(56) **References Cited**

U.S. PATENT DOCUMENTS

3,773,652 A \* 11/1973 Dille et al. ..... 585/265  
3,914,934 A \* 10/1975 Nestor ..... 60/208  
4,251,346 A 2/1981 Dry et al.  
4,318,797 A 3/1982 Jager et al.  
4,330,302 A \* 5/1982 Taylor ..... 44/322  
4,871,444 A 10/1989 Chen et al.  
5,171,916 A 12/1992 Le et al.  
6,274,029 B1 8/2001 Wittenbrink et al.  
6,296,757 B1 10/2001 Wittenbrink et al.  
6,309,432 B1 10/2001 Wittenbrink et al.  
6,392,109 B1 5/2002 O'Rear et al.  
2003/0085153 A1 \* 5/2003 O'Rear ..... 208/63

FOREIGN PATENT DOCUMENTS

WO WO 00/23549 \* 4/2000

WO WO 02/22766 A 3/2002

OTHER PUBLICATIONS

G.C. Feighner, The Manufacture of Detergent Alkylate, Journal American Oil Chemists Society, 1958, pp. 520-524, 35.

Kirk-Othmer, Encyclopedia of Chemical Technology, 3<sup>rd</sup> Edition, vol. 2, 1978, pp. 59-61.

Kirk-Othmer, Encyclopedia of Chemical Technology, 2<sup>nd</sup> completely revised edition, vol. 16, 1968, pp. 581-582.

J. Cummins, M. Yoneyama, Nonene (Propylene Trimer) and Tetramer, SRI International, Chemical Economics Handbook, Aug. 2001 pp. 678.5000A-P.

New solid-bed alkylation technology for LAB, World Surfactants Congress, 4<sup>th</sup>, Barcelona, Jun. 3-7, 1996, pp. 177-189.

Ullmann's Encyclopedia of Industrial Chemistry, 6<sup>th</sup> Completely Revised Edition, 2003, vol. 35, pp. 293-368.

Kirk-Othmer, Encyclopedia of Chemical Technology, 4<sup>th</sup> Edition, 1992, vol. 3, pp. 788-812.

Kirk-Othmer, Encyclopedia of Chemical Technology, 4<sup>th</sup> Edition, 1994, vol. 12, pp. 341-342; 373-388.

Gerhartz, W.; Yamamoto, Y.S., Ullmann's Encyclopedia of Industrial Chemistry, vol. A1, 1985, Weinheim, VCH Verlag., DE, XP002331665, p. 190, col. 1, paragraph 2.1.

Kirk-Othmer, Petroleum Composition, Encyclopedia of Chemical Technology, p. 845 and p. 853, vol. 14, Second Edition, Copyright © 1967 by John Wiley & Sons, Inc.

Kirk-Othmer, Petroleum, Encyclopedia of Chemical Technology, p. 570 and pp. 575-594, vol. 18, Fifth Edition, Copyright © 2006 by John Wiley & Sons, Inc.

Robert A. Meyers, Handbook of Petroleum Refining Processes, pp. 7.21 through 7.32, p. 7.38 and p. 7.40, Second Edition, Copyright © 1967 by The McGraw-Hill Companies, Inc.

\* cited by examiner

*Primary Examiner*—Walter D Griffin

*Assistant Examiner*—Lessanework Seifu

(74) *Attorney, Agent, or Firm*—Laura R. Grunzinger

(57) **ABSTRACT**

A fuel or fuel blendstock for jet, gas turbine, rocket, and diesel engines, particularly jet, rocket, and diesel engines that utilizes components of conventional petroleum not currently utilized for jet, gas turbine, rocket, and diesel fuels, such as benzene, linear, and lightly branched alkanes, that may be alkylated with aromatic moieties to make monoaromatics for use in jet and diesel fuels. Additionally, a fuel having such monoaromatics having multiple desired properties such as higher flash point, low pour point, increased density, better lubricity, aerobic degradability, reduction in toxicity, and additionally can deliver benefits in blendstocks.

**12 Claims, No Drawings**

## 1

FUEL FOR JET, GAS TURBINE, ROCKET  
AND DIESEL ENGINES

## FIELD OF THE INVENTION

The present invention relates to a fuel or fuel blendstock for jet, gas turbine, rocket, and diesel engines, particularly jet, rocket, and diesel engines.

## BACKGROUND OF THE INVENTION

The availability and quality of natural resources for jet, gas turbine, rocket, and diesel fuels presents unique and difficult technical challenges. An identified problem is the increasing demand for jet and diesel fuels for aircraft and for motor vehicles. As quality requirements for fuels are increasing, the ability to produce acceptable fuels from a conventional petroleum barrel of crude is decreasing. Due to the fact that conventional barrels of crude are becoming, on the average, heavier (e.g., more polycyclic) and containing more sulfur, the need for acceptable fuels is an unmet need. At the same time, the drive for cleaner fuels results in highly hydrogenated, less dense fuels that result from processing to remove sulfur and polycyclics such as naphthalenes. It is believed that highly purified conventional fuels and highly paraffinic Fischer-Tropsch fuels are of lower densities, lack seal swelling abilities, and lubricity. Restrictions on gasoline content make available carbon containing components not having any immediate uses, such as benzene and shorter chain hydrocarbons having from five to nine carbon atoms.

Circulating fuel in and around an aircraft commonly provides the sole means of cooling engines, lubes, electronics, wings, etc. of an aircraft. Significantly increased heat loads are an identified problem as fuel economy and performance considerations raise engine temperatures. More flights are using polar routes and therefore fuels must not withstand broader temperature ranges when used. The ability to raise fuel flash point to 60° C. or more while maintaining pour points below -60° C. remains an unmet need. Another desired result of raising flash points above present specifications is desirable to increase chances of surviving crashes or fires when fueling and flying aircraft.

It is also desired to have a flexible and diversified fuel source so that not only are materials for fuels derived from petroleum based components, but may be derived from natural gas, coal, petroleum residue, biomass, and waste feedstocks via syngas. However, such flexibility and diversification is currently not widely available. Therefore, there exists a need to address the issues discussed hereinabove.

## SUMMARY OF THE INVENTION

A fuel composition for use in jets, gas turbines, rockets, or diesel engines comprising:

(a) from about 5% to about 99% by weight of the fuel composition of formula (I)



wherein A is selected from benzene, toluene, xylene, cyclohexane, and mixtures thereof, more preferably A is benzene, toluene, or cyclohexane, most preferably benzene; such that A is non-terminally attached to the L moiety and further such that A is directly connected to the L moiety; R' is selected

## 2

from hydrogen and C<sub>1</sub> to C<sub>3</sub> alkyl; R'' is selected from hydrogen and C<sub>1</sub> to C<sub>3</sub> alkyl; wherein both of R' and R'' are nonterminally attached to the L moiety; the L moiety is a linear acyclic aliphatic hydrocarbyl such that the sum of carbons in the L moiety, R', and R'' is from 5 to 25 carbons;

b) at least about 0.01% of fuel additives; and

(c) about 0% to about 90% of conventional jet, gas turbine, rocket or diesel blendstocks, preferably ultra low sulfur refined petroleum blendstocks or Fischer Tropsch blendstocks.

## DETAILED DESCRIPTION OF THE INVENTION

Restrictions on gasoline content, such as benzene, shorter chain (C<sub>5</sub> to C<sub>9</sub>) linear, and lightly branched alkanes, have made or will make available components which can be used to alkylate aromatics to make monoaromatics used in jet and diesel fuels. The use of monoaromatics as fuels, specifically alkylbenzenes made from benzene and surplus conventional petroleum components or Fischer-Tropsch derived shorter chain (C<sub>5</sub> to C<sub>14</sub>) linear, and lightly branched alkanes, may be beneficial in multiple ways. Use of such benzenes and shorter chain (C<sub>5</sub> to C<sub>14</sub>) linear, and lightly branched alkanes would add to the volume of jet fuel, which is an identified need, while removing undesired materials from gasoline for use in motor vehicles. Additionally the fuel of the present invention has multiple desired properties such as higher flash point, lower pour point, high temperature stability, oxidative stability, increased density, better lubricity, reduction in toxicity in its own right, and can deliver benefits in blendstocks. These identified properties provide improved fuels especially for higher performance aircraft featuring conventional jet, ramjet, scramjet, rocket, or pulse detonation engines and the like.

Shorter paraffinic chainlengths from C<sub>5</sub> to C<sub>9</sub> may be combined with aromatics such as benzene and, optionally, aromatics reduced to cyclohexanes to form a fuel having several desirable attributes for jet, gas turbine, rocket, and diesel fuel. Alkylating benzene with mostly linear olefins and/or olefins from paraffins would be an alternative way of increasing branching of the olefins and/or olefins from paraffins as opposed to hydroisomerization. In other words, the fuel of the present invention presents a viable and cost effective method of increasing branching of low molecular weight Fischer-Tropsch products. The fuel of the present invention may also be derived from non-petroleum feedstocks such as natural gas, coal, tar sands, or oil shale. The diversified production sources listed provide a highly desirable fuel source flexibility.

An identified problem in the jet and diesel fuel area is the ability of a fuel to deliver multiple properties, such as lower pour point, increased lubricity, increased flash point, reduction in toxicity, compatibility in blendstocks with conventional or ultra low sulfur conventional jet, gas turbine, rocket, and/or diesel fuels, among other properties. Additionally, the alkylaromatics may be hydrogenated to alkylcyclohexanes to make fuels capable of providing endothermic cooling in special high performance aircraft engines/airframes of the future.

The fuel of the present invention may also be preferably used as part of a blendstock for use in hydrocarbon fuel-powered equipment, nonlimiting examples such as camp stoves, chainsaw, generators, and the like. Fuels, herein after referred to as "universal battlefield fuel", such as the fuel of the present invention may be used in various hydrocarbon fuel-powered machines. As used herein "hydrocarbon fuel" means gasoline, kerosene, fuel oil, and diesel. Furthermore, higher flash point, increased density, better lubricity of the

fuel of the present invention's alkylaromatics or blends of alkylaromatics with conventional fuels such as highly processed jet fuels or Fischer-Tropsch jet fuels may render the fuel of the present invention more suitable for use in military diesel engines as well, thus improving applicability of universal battlefield fuels. These benefits could also be useful in common vehicle and off-road diesel fuels generally when blended with highly processed conventional or Fischer-Tropsch diesel stocks.

The fuel composition comprises from about 5 wt % to about 99 wt % by weight of the fuel composition of an alkylaromatic or alkylcyclohexane of formula (I):



(I)

wherein the A moiety is selected from an aromatic moiety, a moiety derived from an aromatic moiety, such as cyclohexane, and mixtures thereof. Preferably, the A moiety is benzene, toluene, xylene, cyclohexane, and mixtures thereof, more preferably the A moiety is benzene, toluene, or cyclohexane, most preferably benzene or cyclohexane. The A moiety, such as benzene may be derived from petroleum or coal, such as coal oil. The A moiety is nonterminally attached to the L moiety. The A moiety is also such that it is directly connected to the L moiety, or in other words, there is no methylene moiety between the A moiety and the L moiety.

R' is selected from hydrogen and C<sub>1</sub> to C<sub>3</sub> alkyl. Preferably, R' is hydrogen, methyl or ethyl, more preferably, R' is hydrogen or methyl. R' is nonterminally attached to the L moiety. That is, R' does not add to the overall chain length of the L moiety, but rather, is branching from the L moiety.

R'' is selected from hydrogen and C<sub>1</sub> to C<sub>3</sub> alkyl. Preferably, R'' is hydrogen, methyl or ethyl, more preferably, R'' is hydrogen or methyl. R'' is nonterminally attached to the L moiety. That is, R'' does not add to the overall chain length of the L moiety, but rather, is branching from the L moiety. The fuel of the present invention is such that R' and R'' are selected to achieve a lightly branched alkylaromatic or alkylcyclohexane, further discussed below, having an average of about 1.0 to about 1.5 branches per molecule.

The L moiety is an acyclic aliphatic hydrocarbyl such that L+R'+R'' is from 5 to 25 carbon atoms. In a preferred embodiment of the fuel of the present invention the total carbons of L, R', and R'' is from 5 to 7. In another preferred embodiment of the fuel of the present invention the total carbons of L, R', and R'' is from 8 to 10. In another preferred embodiment of the fuel of the present invention the total carbons of L, R', and R'' is from 10 to 14. In another preferred embodiment of the fuel of the present invention the total carbons of L, R', and R'' is from 5 to 14. The preferred L moiety is: R''—C(—)H(CH<sub>2</sub>)<sub>v</sub>C(—)H(CH<sub>2</sub>)<sub>x</sub>C(—)(CH<sub>2</sub>)<sub>y</sub>—CH<sub>3</sub>, wherein the three C(—) indicate the three carbon atoms where the A moiety, R', and R'' may be attached to formula (II) below:



(II)

wherein R', R'' and the A moiety are hereinbefore defined such that there are no quaternized carbon atoms in the compounds of formula I or formula II.

R''' is selected from C<sub>1</sub> to C<sub>6</sub> alkyl. Preferably R''' is C<sub>1</sub> to C<sub>3</sub> alkyl, more preferably R''' is methyl or ethyl. The numbers of the methylene subunits, v, x and y are each independently integers from 0 to 10 provided that the total number of carbons excluding carbons of the A moiety (e.g., in formula (I), the sum of carbons in L, R', and R''; in formula (II), the sum of carbons in R', R'', R''', and C(—)H(CH<sub>2</sub>)<sub>v</sub>C(—)H(CH<sub>2</sub>)<sub>x</sub>C(—)(CH<sub>2</sub>)<sub>y</sub>—CH<sub>3</sub>) is between 5 and 25 carbon atoms. Therefore, not being limited by example, 2-phenylpentane would equate to formula (I) having the L moiety being a acyclic aliphatic hydrocarbyl having 5 carbon atoms, R' and R'' being hydrogen, and the A moiety being benzene; or formula (II) having v, x, and y being 0, R' and R'' being hydrogen, R''' being a C<sub>1</sub> and the A moiety being benzene.

In the fuel of the present invention, the A moiety is preferably attached to the L moiety in the position which is selected from positions alpha- and beta- to either of the two terminal carbon atoms of the L moiety, preferably the A moiety is attached to the L moiety in position alpha- to a terminal carbon atom of the L moiety. The terms alpha- and beta- mean the carbon atoms that are one and two carbon atoms away, respectively, from the terminal carbon atoms. To better explain this, the structure below shows the two possible alpha-positions and the two possible beta-positions in a general linear hydrocarbon.



Furthermore, in the first aspect of the invention, the fuel composition may have a molar ratio of nonquaternary to quaternary carbon atoms in the L moiety of formula (I) or the combination of R''' and C(—)H(CH<sub>2</sub>)<sub>v</sub>C(—)H(CH<sub>2</sub>)<sub>x</sub>C(—)(CH<sub>2</sub>)<sub>y</sub>—CH<sub>3</sub> moiety of formula (II) of at least about 50:1, and most preferably at least 200:1.

Any of the alkylaromatics, preferably alkylbenzene, may be partially or completely converted to the corresponding alkylcyclohexanes via catalytic hydrogenation, should lower aromaticity or no aromaticity be required of a specific fuel. Such an embodiment is not preferred due to cost consideration for conventional jet, gas turbine, rocket, and/or diesel fuel composition applications. However, conversion to alkylcyclohexanes may be useful in application where extra cost is warranted. Conversion to alkylcyclohexanes may be useful in special aircraft or rocket fuel applications where extra cost is warranted, for example for endothermic cooling properties. The conversion from an alkylaromatic, such as alkylbenzene, to an alkylcyclohexane, may be accomplished by the step of hydrogenating the alkyl aromatic, preferably alkylbenzene, to an alkylcyclohexane.

The fuel of the present invention may deliver one of the properties discussed below; however, it is preferred that the fuel of the present invention delivers multiple benefits.

65 Fuel Density—The fuel of the present invention has a density of at least about 0.700 g/mL, preferably about 0.700 g/mL to about 0.900 g/mL, more preferably from about 0.750

to about 0.860 g/mL. The fuel density may be measured by ASTM D 1298 (API Gravity) or ASTM D 4052 (Digital Density Meter). Fuel density usually is used to predict energy content of a jet fuel composition. Less dense jet fuels have a higher gravimetric energy content (energy per unit weight of fuel), and more dense jet fuels have a higher volumetric energy content (energy per unit volume of fuel). A more dense fuel with a high volumetric energy content is generally preferred.

Fuel economy of diesel fuel is related to the heating value or energy content of the diesel fuel. Heating value per liter or gallon is directly proportional to density when other fuel properties are unchanged. Relative density (RD), also called specific gravity, or API gravity (ASTM D 287), while more conventional reporting methods for density, can easily be determined by one skilled in the art from the density of the fuel of the present invention.

Cetane index may be measured by ASTM D 976 and ASTM D 4737 (four variable equation). The fuel of the present invention when in the form of a diesel fuel has a cetane index at least about 40, preferably from about 40 to about 70. This can be achieved by blending with a paraffinic/isoparaffinic Fischer-Tropsch or highly hydrogenated conventional petroleum diesel stocks. The cetane index is a calculated quantity that is intended to approximate the cetane number, measured by ASTM D 613.

The aromatic content of the fuel of the present invention may be measured by ASTM D 1319 for jet and diesel fuels. Aromaticity for diesel fuels may be measured by ASTM D 5186. It is preferred that the fuel of the present invention is essentially free of polycyclic, particularly polycyclic aromatic substituents, including naphthalenes, alkylnaphthalenes, and tetralins, and is essentially free of unreacted (or free) benzene, toluene, and xylene. As used herein "essentially free" refers to having less than 10 ppm present in the fuel composition of the present invention. Without being limited by a theory, it is believed that the removal of sulfur and polycyclics such as naphthalenes from fuels result in fuels having reduced seal swelling abilities. It is believed that the alkylaromatics, preferably alkylbenzenes of the fuel of the present invention provide seal swelling benefits.

Freeze Point—The freeze point of fuels can be over a wide range of temperatures. Wax crystals are the first indications that a fuel is freezing. After wax crystals are formed, the fuel becomes a slush of fuel and crystals, then forming a solid mass. Freeze point, as used herein, refers to the temperature at which the last wax crystal melts, when warming a fuel that has previously been cooled until wax crystals form. Jet fuels generally are discussed in terms of freeze point. The freeze point measurement for jet fuels employs several standard test methods, including ASTM D 2386 (Referee Method), ASTM D 4305 (Filter Flow), ASTM D 5901 (Automated Optical Method), and ASTM D 5972 (Automatic Phase Transition Method). Jet fuels require pumpability to move from the jet fuel tank to the jet engine. The pumpability of the jet fuel should be more than 4° C. below the freeze point of the jet fuel. Diesel fuels are generally discussed in terms of pour point or cloud point. Cloud point is measured by ASTM D 2500 and Pour Point is measured by ASTM D 97. The pour point of the fuel of the present invention is at least about -40° C., preferably from about -40° C. to about -80° C., preferably from about -47° C. to about -80° C. for jet, rocket, or gas turbine engines. The pour point of the fuel of the present invention is at least about -20° C., preferably about -20° C. to about -80° C. for diesel engines. The pour point of the fuel of the present invention makes it highly desirable for low temperature operability due to good low temperature viscosities.

Low Temperature Operability may be measured by IP 309 (CFPP) or ASTM D 4539 (FTFT). Without being limited by a theory, it is believed that the low pour point of the fuel of the present invention, despite the molecular weight of the fuel of the present invention, also translates into acceptable flash point, as discussed below.

Flash Point—The fuel of the present invention has a flash point from about 30° C. to about 145° C., preferably from about 60° C. to about 145° C. Flash point for jet fuel may be measured by ASTM D 56 (Tag Closed Tester or Referee Method) or ASTM D 3828 (Small Scale Closed Tester). Flash point for diesel fuel may be measured by ASTM D 93 (Pensky-Marten Closed Cup Tester). A raised flash point will be especially useful for hot fueling of fuel tanks. As used herein "hot fuel" means refilling the fuel tank of a machine such as an aircraft or motorized vehicle that is running or still hot from being run. Higher flash points of the fuels of the present invention may also allow for reduction in fueling time critical in military and jumbo civilian aircraft. Another desired result of raising flash points above present specifications is desirable to increase safety, reduce the danger of fuel tank explosions, and increasing chances of surviving crashes or fires when fueling and flying aircraft.

Thermal Stability—the fuel of the present invention may demonstrate improved thermal stability, which is important to jet, gas turbine, rocket, and diesel fuels as fuels are used to cool engines and other parts of the jet engine, gas turbine, rocket engine, and diesel engines. Without stability at higher temperatures, gum and particulate formation increases causing damage to engines. Standardized testing includes Jet Fuel Thermal Oxidation Tester (JFTOT) (ASTM D3241). Diesel fuel thermal stability is measured by Octel/Dupont F21-150° C. Accelerated Fuel Oil stability Test. The fuel of the present inventions should meet or exceed conventional fuel thermal stability standards. Thermal stability may be measured in the presence of oxygen (oxidative stability) or the absence of oxygen.

Lubricity—Lubricity of jet, gas turbine, rocket, and diesel fuel is impacted by the aromatic content as well as the oxygen, nitrogen, and sulfur containing compound content. As governmental regulations seek to decrease the content of aromatics, oxygen, nitrogen, and sulfur containing compounds, lubricity of the fuel is decreased. The fuel of the present invention preferably demonstrates self-lubing properties alone or in a blendstock. Lubricity for jet fuel is measured by ASTM D 5001 (BOCLE Test). ASTM D 975 measures hydrodynamic lubrication in diesel fuels.

Particulate Reduction/Luminosity Reduction—Particulates are formed by incomplete combustion of fuels. These particulates are harmful to the jet and diesel engines mechanically, and can form the smoke emitted from engines. Polycyclics are the major cause of smoke and soot produced by fuels; however, the fuel of the present invention is essentially free of polycyclic aromatics and therefore minimizes the formation of harmful particulates. The fuel of the present invention, when in the form of a jet fuel, has a minimum smoke point of at least about 20 mm. Smoke Point is measured by ASTM D 1322. With jet fuels these particulates can become incandescent under the high temperature and pressure conditions of the combustion section. This too may lead to cracks and premature engine failures.

Diesel fuels require the ash content to have a maximum of 100 ppm. ASTM D 482 measures ash content in diesel fuels.

Other fuel properties may be required by known fuel specifications that have not been discussed above. Properties such as antistatic, corrosion resistance, anti-growth, oxidative stability, and thermal stability in the absence of oxygen, may

also be delivered by the fuel of the present invention. The fuel of the present invention, without being limited by a theory, is believed to have less inherent toxicity compared to conventional fuels and is believed to be aerobically more environmentally friendly than conventional fuels.

The fuel of the present invention may be derived from several different starting materials including olefins, paraffins, and alcohols. The fuel of the present invention utilizes not only linear alkylaromatics and linear alkylcyclohexanes, but also lightly branched alkylaromatics and alkylcyclohexanes.

#### Linear Alkylaromatics

Linear alkylaromatics, such as alkylbenzene, can be made by the alkylation of an aromatic moiety, preferably benzene, by a Friedel-Crafts reaction, similar to the manufacturing process utilized for detergents, with adjustments for potential inclusion of carbon chain lengths as short as C<sub>5</sub>. Starting materials of alkylation process include n-paraffins, n-olefins, and mixtures thereof and aromatic materials including benzene, toluene, xylene, and mixtures thereof.

The n-paraffins, n-olefins, and mixtures thereof may undergo steps prior to the alkylation process to produce linear materials suitable for the alkylation step with the aromatic materials. For example, paraffins may be converted into chloroparaffins and alkylated in the presence of aluminum chloride. The chloroparaffins may also be converted to linear olefins and alkylated in the presence of aluminum chloride. Paraffins may also be directly converted to linear olefins via the PACOL® process, by UOP Inc., followed by selective hydrogenation (DEFINE® Process, by UOP Inc.), then used in the alkylation process.

The selected starting materials including n-paraffins, n-olefins, and mixtures thereof, and aromatic starting materials, such as benzene, toluene, xylene, and mixtures thereof are mixed with an alkylation catalyst to form the alkylaromatics via an alkylation step. Aluminum chloride and hydrogen fluoride may be used as alkylation catalysts in the alkylation process. Further discussion of such process may be found in Ullmann's Encyclopedia of Industrial Chemistry, Vol. 35, pages 293-368, entitled "Surfactants". Such procedures are also discussed in Kirk-Othmer Encyclopedia of Chemical Technology, 3<sup>rd</sup> Edition, Vol. 2, pages 50-70, in the article entitled "Alkylation". See also U.S. Pat. No. 5,344,997, U.S. Pat. No. 5,196,574, U.S. Pat. No. 5,334,793, and U.S. Pat. No. 5,245,094.

Solid-Bed Alkylation for producing linear alkylaromatics, known as the DETAL® process, which was co-developed by UOP Inc. and Petresa Inc., may also be used to produce the linear alkylaromatics, preferably alkylbenzene for the fuel of the present invention. Further discussion of the DETAL® process is found in World Surfactants Congress, 4th, Barcelona, Jun. 3-7, 1996 (1996), pages 117-189 (ISBN 0-85404-751-4). The DETAL® process may further comprise the use of the DEFINE® process, licensed by UOP Inc., for selective hydrogenation converting diolefins to monoolefins, which then may be used in the alkylation process. The DETAL® process may further comprise the PEP® process, licensed by UOP, for adsorption and fractionation of aromatic compounds undesired in the fuel of the present invention. Uses of such processes are preferred in the fuel of the present invention.

#### Lightly Branched Alkylaromatics

The fuel of the present invention may also comprise lightly branched alkylaromatics and alkylcyclohexanes. As used herein "lightly branched" refers to the branching on olefins or olefins derived from paraffins utilized as feedstocks for the

alkyl moiety of the fuel of the present invention (e.g., formula (I): L, R' and R''), wherein the olefins or olefins derived from paraffins comprise selected short chain (C<sub>1</sub> to C<sub>4</sub> alkyl) branches such that about 20 wt % to about 100 wt %, by weight of the alkylaromatic and/or alkylcyclohexane molecules have an average of 1.0 to about 1.5 branches per molecule. As used herein "linear" refers to the alkyl moiety of the fuel of the present invention (e.g., formula (I): L, R' and R'') having less than about 5 wt % of one methyl branch per molecule. The fuel of the present invention also includes a mixture of linear and lightly branched alkylaromatics, a mixture of linear and/or lightly branched alkylcyclohexane, and mixtures thereof.

Several processes may be used to make lightly branched alkylaromatics prior to the alkylation process. Linear reduction of olefins and paraffins via skeletal isomerization followed by alkylation is a process discussed in WO 99/05082. Processes utilizing alcohols and alkylation of aromatic moieties are also applicable to the fuel of the present invention.

Lightly Branched Modification via Skeletal Isomerization of Olefin—Preferred starting-material olefins for lightly branched modification of olefins by skeletal isomerization herein are alpha-olefins. Suitable olefins can in general be obtained from any source, including those made from kerosene processed through the PACOL® and OLEX® processes of UOP Inc. or less preferably via the older Shell Inc. (CDC) process; alpha-olefins generated by ethylene polymerization, for example by the Shell, Gulf/Chevron, or Amoco (formerly Ethyl Corp.) processes; alpha olefins derived from cracked wax; alpha-olefins derived from Fischer-Tropsch syntheses, or internal olefins from Shell's SHOP® process.

Skeletal isomerization of olefins utilized herein can, in general, be accomplished in any manner known in the art. Suitable constrained skeletal isomerization catalysts are known for various purposes and include those selected from the group consisting of zeolites and silicoaluminophosphates, including, but not limited to: ALPO-31®, SAPO-11®, SAPO-31® and SAPO-41®; preferably SAPO-11®. See U.S. Pat. No. 5,510,306. The preferred catalysts comprise substantially only zeolites. Further examples are discussed in WO 99/05082.

Skeletal isomerization of linear paraffin—Preferred starting-material paraffins for delinearization of paraffins by skeletal isomerization herein are linear paraffins. Suitable paraffins can more generally be obtained from any source, such as those derived from kerosene treated by UOP's MOLEX® process. In general, any catalyst suitable for alkyl branching, preferably methyl branching, of a linear paraffin is useful in the instant process. Preferred skeletal isomerization catalysts for this step include (i) zeolites having ferrierite isotopic framework structure (more preferably H-ferrierites); (see for example U.S. Pat. No. 5,510,306) and (ii) ALPO-31®, SAPO-11®, SAPO-31® and SAPO-41®. Lightly branched paraffins from Fischer-Tropsch are preferred materials.

Dehydrogenation of skeletally isomerized paraffin—In general, dehydrogenation of the skeletally isomerized paraffin in the instant process can be accomplished using any of the well-known dehydrogenation catalyst systems. Dehydrogenation can be conducted in presence of hydrogen gas and commonly a precious metal catalyst is present though alternatively non-hydrogen, precious-metal free dehydrogenation systems such as a zeolite/air system can be used with no precious metals present. As is well known, dehydrogenation can be complete or partial, more preferably partial. When partial, dehydrogenation step forms a mixture of olefin and

unreacted paraffin. Such mixture is a suitable material for the alkylation step of the alkylation process.

#### Use of Alcohols

Alternatively, a process may provide an alcohol or alcohol mixture having molecular weight of from about 144 to about 242. In general, suitable alcohol can be made by selective hydroformylation of Fischer-Tropsch olefins, or skeletally isomerized linear olefins, by positionally nonselectively hydroformylating linear olefins and by reactions of Grignard reagents or suitable equivalent organometallics such as organolithium reagents, with methyl alkyl ketones. The alcohol may be used in the alkylation step to alkylate the aromatic moiety, in the manner discussed above.

Alcohols via Grignard technique—In the Grignard technique, a mixture of ketones such as 2-hexanone, 2-heptanone, and 2-octanone at a 2:2:1 mole ratio are reacted with an alkyl Grignard reagent such as hexylmagnesium bromide. On workup, a mixture of alcohols, in the case of this specific illustration 5-methyl-5-undecanol, 6-methyl-6-dodecanol and 7-methyl-7-tridecanol, is secured.

Despite the seemingly counterintuitive use of alcohols rather than olefins to make the fuel of the present invention, the process has some unique advantages, for example in that alcohols can be dehydrated, isomerized and alkylated herein in one step through the use of a catalyst such as a zeolite with acidic sites within the catalyst. Moreover, alcohols can be conveniently made and used to conduct tailored batch syntheses of the alkyl aromatics for use in the fuel of the present invention at relatively small scales using commercially available alcohols such as natural, Ziegler, or NEODOL® alcohols, even when the corresponding olefins are not readily available in relatively small quantities.

Mixtures of linear alkylaromatics, linear alkylcyclohexane, lightly branched alkylaromatic, lightly branched alkylcyclohexane, and mixtures thereof may comprise the fuel of the present invention. Fischer-Tropsch processes are a preferable source of the mixtures of linear and/or lightly branched alkylaromatics, preferably linear and/or lightly branched alkylbenzene. These mixtures may be obtained from several points in Fischer Tropsch (F.T.) process. Examples of different points include obtaining the desired materials from straight run F.T. processes, hydroisomerate/hydrocrackates from F.T. middles distillates, hydrocrackates from F.T. lube making, and hydrocrackates from F.T. wax. The hydrocrackates yield paraffins, which require an additional step of dehydrogenation to olefins, as defined above in the linear alkylaromatic section. The use of hydrocrakages from F.T. technology is as used in making alkylbenzenes for detergents. Alternatively, cracking could replace hydrocracking in these steps to make olefins directly for use as fuels of the present invention. Steam or nitrogen cracking of waxes is known in alkylbenzene processes and may be utilized in making the fuel of the present invention. F.T. plants will produce adequate amounts of steam and nitrogen to practice the cracking process to produce the fuel of the present invention.

#### Alkylation

The process for making lightly branched alkylaromatics for use in the fuel of the present invention further includes the step after the modification to form lightly branched olefins and/or paraffins, a monoalkylation step of reacting the lightly branched olefin and/or paraffin with an aromatic moiety selected from benzene, toluene, xylene, and mixtures thereof, preferably benzene.

#### Alkylation Catalyst

A suitable alkylation catalyst herein may be selected from shape-selective moderately acidic alkylation catalysts, pref-

erably zeolitic. The zeolite in such catalysts for the alkylation step is preferably selected from the group consisting of mordenite, ZSM-4®, ZSM-12®, ZSM-20®, offretite, gmelinite and zeolite beta in at least partially acidic form. Particularly preferred alkylation catalysts herein include the acidic mordenite catalysts ZEOCAT® FM-8/25H available from Zeochem; CBV 90 A®, available from Zeolyst International, and LZM-8® available from UOP Chemical Catalysts. A further discussion of suitable alkylation catalysts is found in WO 99/05082. Further discussions on the process may be found in WO 99/05084 and WO 00/12451.

#### Fuel Additives

The fuel of the present invention may optionally comprise at least about 0.01 wt %, preferably from about 0.01% to about 5%, preferably from about 0.1% to about 5% by weight of the fuel composition of a fuel additive.

Jet fuel additives such as antioxidants, metal deactivators, electrical conductivity or static dissipaters, corrosion inhibitors, lubricity improvers, fuel system icing inhibitors, biocides, thermal stability additives, soot/particulate reduction agents, and any combination thereof may be added to the fuel of the present invention. A discussion of these additives may be found in Kirk Othmer Encyclopedia of Chemical Technology, Fourth Edition, Volume 3, pages 788-812, entitled "Aviation and Other Gas Turbine Fuels", specifically, page 795, Table 5.

Diesel Fuel Additives may include cetane index improvers such as 2-ethylhexyl nitrate (EHN), injector cleaning additives, lubricity additives (i.e., fatty acids and esters), smoke suppressants (i.e., organometallic compounds), fuel handling additives such as antifoam additives (i.e., organosilicone compounds), de-icing additives (i.e., low molecular weight alcohols or glycols), low temperature operability additives; drag reducing additives (i.e., high molecular weight polymers) antioxidants such as phenylenediamine, stabilizers, metal deactivators (e.g., chelants), dispersants, biocides, demulsifier, corrosion inhibitors, and any combinations thereof may comprise the fuels of the fuel of the present invention. A discussion of diesel fuel additives may be found in Kirk Othmer Encyclopedia of Chemical Technology, Fourth Edition, Volume 12, pages 341-388, entitled "Gasoline and other Motor Fuels", specifically pages 379-81.

#### Conventional Jet or Diesel Blendstocks

The fuel of the present invention may optionally comprise conventional jet or diesel blendstocks. Preferably, these blendstocks are low sulfur blendstocks or Fischer Tropsch blendstocks. As used herein "conventional" refers to jet or diesel fuels commercially available or known in the art.

The fuel of the present invention comprises no greater than 95 wt %, preferably from about 0 wt % to 90 wt %, preferably from 0 wt % to 80 wt %, preferably from 0 wt % to about 50 wt % by weight of the fuel composition of convention jet or diesel fuels.

#### Methods of Use

The present invention further comprises a method of powering a diesel engine through the burning of a fuel comprising the steps of compressing air in the diesel engine, injecting the fuel of the present invention, igniting the air and fuel to form a burning mixture.

The present invention further comprises a method of powering a jet or gas turbine engine through the burning of a fuel comprising the steps of drawing air from the front of the jet engine or gas turbine into the jet engine or gas turbine, mixing the air with the fuel of Claim 1, igniting the air and fuel mixture to form a burning mixture, and ejecting the burning mixture out of the back of the jet engine or gas turbine.

## 11

The present invention further comprises a method of powering a rocket through the burning of a fuel comprising the steps of mixing the fuel of Claim 1 with an oxidant such as oxygen or nitrous oxide, and mixture thereof, igniting the oxygen, nitrous oxide, and mixtures thereof and fuel to form a burning mixture, and ejecting the burning mixture from the rocket. The present invention further comprises, although not preferred, a method of powering a vehicle having a power system consisting of a at least 70 MPa direct injection diesel engine, preferably of the common rail type, or a hybrid power system comprising the engine and an electric motor comprising a step of combusting the fuel composition of the present invention.

The present invention further relates to a method for powering a ramjet or scramjet. A ramjet has no moving parts and achieves compression of intake air by the forward speed of the air vehicle. Air entering the intake of a supersonic aircraft is slowed by aerodynamic diffusion created by the inlet and diffuser to velocities comparable to those in a turbojet augmentor. The expansion of hot gases after fuel injection and combustion accelerates the exhaust air to a velocity higher than that at the inlet and creates positive push. Scramjet is an acronym for Supersonic Combustion Ramjet. The scramjet differs from the ramjet in that combustion takes place at supersonic air velocities through the engine. Hydrogen is normally the fuel used. Pulse detonation engines are also intended to be included in the method of the present invention. The method of the present invention comprises the steps of decomposing the fuel composition of the present invention, preferably via catalytically dehydrogenating, into hydrocarbon components and hydrogen, and cooling of adjacent engine and airframe parts through endothermic cooling. The hydrocarbon components and hydrogen are then burned. The burning hydrogen is also used to maintain flame under ramjet or scramjet conditions.

## EXAMPLE 1

## Linear Alkylbenzene Prepared Via Alkylation with Alkyl Chlorides

A homologous mixture of  $C_5$ - $C_{25}$  linear alkanes is reacted with gaseous chlorine at 100-140° C. in a chlorination tower to a conversion of 30 mol %. Suitable reactor materials are lead, silver, or enamel; iron is not suitable. The hydrogen chloride release in the reaction  $RH + Cl_2 \rightarrow RCl + HCl$  escapes from the chlorination tower and is washed in a countercurrent fashion with fresh alkane. The alkyl chlorides and unreacted paraffin are passed to the alkylation stage. The alkylation catalyst, aluminum chloride, is a liquid complex compound in the reaction mixture and containing up to containing up to 35 wt % aluminum chloride. The alkylation is preferentially carried out in glass-lined reaction towers at 80° C. Benzene is added in molar excess and hydrogen chloride is released in stoichiometric amounts according to the equation  $RCl + C_6H_6 \rightarrow RC_6H_5 + HCl$ . The catalyst complex is separated out and unreacted benzene and paraffin preferably are removed.

## EXAMPLE 2

## Linear Alkylbenzene Prepared Via Alkylation with Olefins

Dehydrogenate  $C_5$ - $C_{25}$  n-alkanes at ca. 500° C. with a slight hydrogen excess pressure of ca. 300 kPa (3 bar) over a fixed-bed of modified platinum catalyst on aluminum oxide. See U.S. Pat. No. 5,672,797 and U.S. Pat. No. 5,962,760,

## 12

assigned to UOP Inc., for further discussion regarding suitable catalysts. The alkane conversion is held at 1-15 wt % to minimize further dehydrogenation to diolefins and aromatics. Optionally, hydrogen released from the reaction is recycled to the dehydrogenation reactor or connected to a reactor for the selective hydrogenation of diolefins to monoolefins (DEFINE® process). The dehydrogenation product, containing 10-15 wt % monoolefins is passed to the alkylation reaction. Benzene and hydrofluoric acid are mixed with the dehydrogenation product at <50° C. with intensive cooling. The acid catalyst is removed and the product may be distilled to obtain the desired products for use in the fuel of the present invention.

## EXAMPLE 3

## Lightly Branched Alkylbenzene Prepared Via Skeletally Isomerized Linear Olefin

Step (a): At Least Partially Reducing the Linearity of an Olefin (by Skeletal Isomerization of Olefin Preformed to Chainlengths Suitable for Fuel Compositions)

A mixture of 1-decene, 1-undecene, 1-dodecene and 1-tridecene (for example available from Chevron) at a weight ratio of 1:2:2:1 is passed over a Pt-SAPO catalyst at 220° C. and any suitable LHSV, for example 1.0. The catalyst is prepared in the manner of Example 1 of U.S. Pat. No. 5,082,956. See WO 95/21225, e.g., Example 1 and the specification thereof. The product is a skeletally isomerized lightly branched olefin having a range of chain lengths suitable for making an alkylbenzene fuel composition. More generally the temperature in this step can be from about 200° C. to about 400° C., preferably from about 230° C. to about 320° C. The pressure is typically from about 0.205 MPa (15 psig) to about 13.9 MPa (2000 psig), preferably from about 0.205 MPa (15 psig) to about 7.0 MPa (1000 psig), more preferably from about 0.205 MPa (15 psig) to about 4.24 MPa (600 psig). Hydrogen is a useful pressurizing gas for the present example. The space velocity (LHSV or WHSV) is suitably from about 0.05 to about 20. Low pressure and low hourly space velocity provide improved selectivity, more isomerization and less cracking. Distill to remove any volatiles boiling at up to 40° C./1.33 kPa (10 mmHg).

Step (b): Using the Product of Step (a) for Alkyling an Aromatic Moiety

To a glass autoclave liner is added 1 mole equivalent of the lightly branched olefin mixture produced in step (a), 20 mole equivalents of benzene and 20 wt % based on the olefin mixture of a shape selective zeolite catalyst (acidic mordenite catalyst ZEOCA® FM-8/25H). The glass liner is sealed inside a stainless steel rocking autoclave. The autoclave is purged twice with 1.83 MPa (250 psig)  $N_2$ , and then charged to 7.0 MPa (1000 psig)  $N_2$ . With mixing, the mixture is heated to 170-190° C. for 14-15 hours at which time it is then cooled and removed from the autoclave. The reaction mixture is filtered to remove catalyst and is concentrated by distilling off unreacted starting-materials and/or impurities (e.g., benzene, olefin, paraffin, trace materials, with useful materials being recycled if desired) to obtain a clear near-colorless liquid product.

## 13

## EXAMPLE 4

Lightly Branched Alkylbenzene Prepared Via  
Skeletal Isomerization of Paraffin

## Step (a i)

A mixture of n-undecane, n-dodecane, n-tridecane, 1:3:1 wt., is isomerized over Pt-SAPO-11 for a conversion better than 90 wt % at a temperature of about 300-340° C., at about 7.0 MPa (1000 psig) under hydrogen gas, with a weight hourly space velocity in the range 2-3 and 30 moles H<sub>2</sub>/mole hydrocarbon. More detail of such an isomerization is given by S. J. Miller in Microporous Materials, Vol. 2., (1994), 439-449. In further examples, the linear starting paraffin mixture can be the same as used in conventional linear alkyl benzene manufacture. Distill to remove any volatiles boiling at up to 40° C./1.33 kPa (10 mmHg).

## Step (a ii)

The paraffin of step (a i) can be dehydrogenated using conventional methods. See, for example, U.S. Pat. No. 5,012,021, Apr. 30, 1991 or U.S. Pat. No. 3,562,797, Feb. 9, 1971. A suitable dehydrogenation catalyst is any of the catalysts disclosed in U.S. Pat. Nos. 3,274,287; 3,315,007; 3,315,008; 3,745,112; 4,430,517; and 3,562,797. For purposes of the present example, dehydrogenation is in accordance with U.S. Pat. No. 3,562,797. The catalyst is zeolite A. The dehydrogenation is conducted in the vapor phase in presence of oxygen (paraffin:dioxygen 1:1 molar). The temperature is in range 450° C.-550° C. Ratio of grams of catalyst to moles of total feed per hour is 3.9:1.

## Step (b): Alkylating the Product of Step (a) Using an Aromatic Hydrocarbon

To a glass autoclave liner is added 1 mole equivalent of the mixture of step (a), 5 mole equivalents of benzene and 20 wt %, based on the olefin mixture, of a shape selective zeolite catalyst (acidic mordenite catalyst ZEOCAT® FM-8/25H). The glass liner is sealed inside a stainless steel, rocking autoclave. The autoclave is purged twice with 1.83 MPa (250 psig) N<sub>2</sub>, and then charged to 7.0 MPa (1000 psig) N<sub>2</sub>. With mixing, the mixture is heated to 170-190° C. overnight for 14-15 hours, at which time it is then cooled and removed from the autoclave. The reaction mixture is filtered to remove catalyst. Benzene and any unreacted paraffins are distilled and recycled. A clear colorless or nearly colorless liquid product is obtained.

## EXAMPLE 5

Lightly Branched Alkylbenzene Prepared Via  
Specific Tertiary Alcohol Mixture from a Grignard  
Reaction

A mixture of 5-methyl-5-undecanol, 6-methyl-6-dodecanol and 7-methyl-7-tridecanol is prepared via the following Grignard reaction. A mixture of 28 g of 2-hexanone, 28 g of 2-heptanone, 14 g of 2-octanone and 100 g of diethyl ether are added to an addition funnel. The ketone mixture is then added dropwise over a period of 1.75 hours to a nitrogen blanketed stirred three neck round bottom flask, fitted with a reflux condenser and containing 350 mL of 2.0 M hexylmagnesium bromide in diethyl ether and an additional 100 mL of diethyl ether. After the addition is complete, the reaction mixture is stirred an additional 1 hour at 20° C. The reaction mixture is then added to 600 g of a mixture of ice and water with stirring. To this mixture is added 228.6 g of 30% sulfuric acid solution. The resulting two liquid phases are added to a separatory

## 14

funnel. The aqueous layer is drained and the remaining ether layer is washed twice with 600 mL of water. The ether layer is then evaporated under vacuum to yield 115.45 g of the desired alcohol mixture. A 100 g sample of the light yellow alcohol mixture is added to a glass autoclave liner along with 300 mL of benzene and 20 g of a shape selective zeolite catalyst (acidic mordenite catalyst ZEOCAT® FM-8/25H). The glass liner is sealed inside a stainless steel, rocking autoclave. The autoclave is purged twice with 1.83 MPa (250 psig) N<sub>2</sub>, and then charged to 7.0 MPa (1000 psig) N<sub>2</sub>. With mixing, the mixture is heated to 170° C. overnight for 14-15 hours at which time it is then cooled and removed from the autoclave. The reaction mixture is filtered to remove catalyst and concentrated by distilling off the benzene, which is dried and recycled. A clear colorless or nearly colorless lightly branched olefin mixture is obtained.

50 5 10 15 20 25 30 35 40 45 50 55 60 65 70 75 80 85 90 95 100 105 110 115 120 125 130 135 140 145 150 155 160 165 170 175 180 185 190 195 200 205 210 215 220 225 230 235 240 245 250 255 260 265 270 275 280 285 290 295 300 305 310 315 320 325 330 335 340 345 350 355 360 365 370 375 380 385 390 395 400 405 410 415 420 425 430 435 440 445 450 455 460 465 470 475 480 485 490 495 500 505 510 515 520 525 530 535 540 545 550 555 560 565 570 575 580 585 590 595 600 605 610 615 620 625 630 635 640 645 650 655 660 665 670 675 680 685 690 695 700 705 710 715 720 725 730 735 740 745 750 755 760 765 770 775 780 785 790 795 800 805 810 815 820 825 830 835 840 845 850 855 860 865 870 875 880 885 890 895 900 905 910 915 920 925 930 935 940 945 950 955 960 965 970 975 980 985 990 995 1000 1005 1010 1015 1020 1025 1030 1035 1040 1045 1050 1055 1060 1065 1070 1075 1080 1085 1090 1095 1100 1105 1110 1115 1120 1125 1130 1135 1140 1145 1150 1155 1160 1165 1170 1175 1180 1185 1190 1195 1200 1205 1210 1215 1220 1225 1230 1235 1240 1245 1250 1255 1260 1265 1270 1275 1280 1285 1290 1295 1300 1305 1310 1315 1320 1325 1330 1335 1340 1345 1350 1355 1360 1365 1370 1375 1380 1385 1390 1395 1400 1405 1410 1415 1420 1425 1430 1435 1440 1445 1450 1455 1460 1465 1470 1475 1480 1485 1490 1495 1500 1505 1510 1515 1520 1525 1530 1535 1540 1545 1550 1555 1560 1565 1570 1575 1580 1585 1590 1595 1600 1605 1610 1615 1620 1625 1630 1635 1640 1645 1650 1655 1660 1665 1670 1675 1680 1685 1690 1695 1700 1705 1710 1715 1720 1725 1730 1735 1740 1745 1750 1755 1760 1765 1770 1775 1780 1785 1790 1795 1800 1805 1810 1815 1820 1825 1830 1835 1840 1845 1850 1855 1860 1865 1870 1875 1880 1885 1890 1895 1900 1905 1910 1915 1920 1925 1930 1935 1940 1945 1950 1955 1960 1965 1970 1975 1980 1985 1990 1995 2000 2005 2010 2015 2020 2025 2030 2035 2040 2045 2050 2055 2060 2065 2070 2075 2080 2085 2090 2095 2100 2105 2110 2115 2120 2125 2130 2135 2140 2145 2150 2155 2160 2165 2170 2175 2180 2185 2190 2195 2200 2205 2210 2215 2220 2225 2230 2235 2240 2245 2250 2255 2260 2265 2270 2275 2280 2285 2290 2295 2300 2305 2310 2315 2320 2325 2330 2335 2340 2345 2350 2355 2360 2365 2370 2375 2380 2385 2390 2395 2400 2405 2410 2415 2420 2425 2430 2435 2440 2445 2450 2455 2460 2465 2470 2475 2480 2485 2490 2495 2500 2505 2510 2515 2520 2525 2530 2535 2540 2545 2550 2555 2560 2565 2570 2575 2580 2585 2590 2595 2600 2605 2610 2615 2620 2625 2630 2635 2640 2645 2650 2655 2660 2665 2670 2675 2680 2685 2690 2695 2700 2705 2710 2715 2720 2725 2730 2735 2740 2745 2750 2755 2760 2765 2770 2775 2780 2785 2790 2795 2800 2805 2810 2815 2820 2825 2830 2835 2840 2845 2850 2855 2860 2865 2870 2875 2880 2885 2890 2895 2900 2905 2910 2915 2920 2925 2930 2935 2940 2945 2950 2955 2960 2965 2970 2975 2980 2985 2990 2995 3000 3005 3010 3015 3020 3025 3030 3035 3040 3045 3050 3055 3060 3065 3070 3075 3080 3085 3090 3095 3100 3105 3110 3115 3120 3125 3130 3135 3140 3145 3150 3155 3160 3165 3170 3175 3180 3185 3190 3195 3200 3205 3210 3215 3220 3225 3230 3235 3240 3245 3250 3255 3260 3265 3270 3275 3280 3285 3290 3295 3300 3305 3310 3315 3320 3325 3330 3335 3340 3345 3350 3355 3360 3365 3370 3375 3380 3385 3390 3395 3400 3405 3410 3415 3420 3425 3430 3435 3440 3445 3450 3455 3460 3465 3470 3475 3480 3485 3490 3495 3500 3505 3510 3515 3520 3525 3530 3535 3540 3545 3550 3555 3560 3565 3570 3575 3580 3585 3590 3595 3600 3605 3610 3615 3620 3625 3630 3635 3640 3645 3650 3655 3660 3665 3670 3675 3680 3685 3690 3695 3700 3705 3710 3715 3720 3725 3730 3735 3740 3745 3750 3755 3760 3765 3770 3775 3780 3785 3790 3795 3800 3805 3810 3815 3820 3825 3830 3835 3840 3845 3850 3855 3860 3865 3870 3875 3880 3885 3890 3895 3900 3905 3910 3915 3920 3925 3930 3935 3940 3945 3950 3955 3960 3965 3970 3975 3980 3985 3990 3995 4000 4005 4010 4015 4020 4025 4030 4035 4040 4045 4050 4055 4060 4065 4070 4075 4080 4085 4090 4095 4010 4015 4020 4025 4030 4035 4040 4045 4050 4055 4060 4065 4070 4075 4080 4085 4090 4095 4100 4105 4110 4115 4120 4125 4130 4135 4140 4145 4150 4155 4160 4165 4170 4175 4180 4185 4190 4195 4200 4205 4210 4215 4220 4225 4230 4235 4240 4245 4250 4255 4260 4265 4270 4275 4280 4285 4290 4295 4300 4305 4310 4315 4320 4325 4330 4335 4340 4345 4350 4355 4360 4365 4370 4375 4380 4385 4390 4395 4400 4405 4410 4415 4420 4425 4430 4435 4440 4445 4450 4455 4460 4465 4470 4475 4480 4485 4490 4495 4500 4505 4510 4515 4520 4525 4530 4535 4540 4545 4550 4555 4560 4565 4570 4575 4580 4585 4590 4595 4600 4605 4610 4615 4620 4625 4630 4635 4640 4645 4650 4655 4660 4665 4670 4675 4680 4685 4690 4695 4700 4705 4710 4715 4720 4725 4730 4735 4740 4745 4750 4755 4760 4765 4770 4775 4780 4785 4790 4795 4800 4805 4810 4815 4820 4825 4830 4835 4840 4845 4850 4855 4860 4865 4870 4875 4880 4885 4890 4895 4900 4905 4910 4915 4920 4925 4930 4935 4940 4945 4950 4955 4960 4965 4970 4975 4980 4985 4990 4995 5000 5005 5010 5015 5020 5025 5030 5035 5040 5045 5050 5055 5060 5065 5070 5075 5080 5085 5090 5095 5100 5105 5110 5115 5120 5125 5130 5135 5140 5145 5150 5155 5160 5165 5170 5175 5180 5185 5190 5195 5200 5205 5210 5215 5220 5225 5230 5235 5240 5245 5250 5255 5260 5265 5270 5275 5280 5285 5290 5295 5300 5305 5310 5315 5320 5325 5330 5335 5340 5345 5350 5355 5360 5365 5370 5375 5380 5385 5390 5395 5400 5405 5410 5415 5420 5425 5430 5435 5440 5445 5450 5455 5460 5465 5470 5475 5480 5485 5490 5495 5500 5505 5510 5515 5520 5525 5530 5535 5540 5545 5550 5555 5560 5565 5570 5575 5580 5585 5590 5595 5600 5605 5610 5615 5620 5625 5630 5635 5640 5645 5650 5655 5660 5665 5670 5675 5680 5685 5690 5695 5700 5705 5710 5715 5720 5725 5730 5735 5740 5745 5750 5755 5760 5765 5770 5775 5780 5785 5790 5795 5800 5805 5810 5815 5820 5825 5830 5835 5840 5845 5850 5855 5860 5865 5870 5875 5880 5885 5890 5895 5900 5905 5910 5915 5920 5925 5930 5935 5940 5945 5950 5955 5960 5965 5970 5975 5980 5985 5990 5995 6000 6005 6010 6015 6020 6025 6030 6035 6040 6045 6050 6055 6060 6065 6070 6075 6080 6085 6090 6095 6100 6105 6110 6115 6120 6125 6130 6135 6140 6145 6150 6155 6160 6165 6170 6175 6180 6185 6190 6195 6200 6205 6210 6215 6220 6225 6230 6235 6240 6245 6250 6255 6260 6265 6270 6275 6280 6285 6290 6295 6300 6305 6310 6315 6320 6325 6330 6335 6340 6345 6350 6355 6360 6365 6370 6375 6380 6385 6390 6395 6400 6405 6410 6415 6420 6425 6430 6435 6440 6445 6450 6455 6460 6465 6470 6475 6480 6485 6490 6495 6500 6505 6510 6515 6520 6525 6530 6535 6540 6545 6550 6555 6560 6565 6570 6575 6580 6585 6590 6595 6600 6605 6610 6615 6620 6625 6630 6635 6640 6645 6650 6655 6660 6665 6670 6675 6680 6685 6690 6695 6700 6705 6710 6715 6720 6725 6730 6735 6740 6745 6750 6755 6760 6765 6770 6775 6780 6785 6790 6795 6800 6805 6810 6815 6820 6825 6830 6835 6840 6845 6850 6855 6860 6865 6870 6875 6880 6885 6890 6895 6900 6905 6910 6915 6920 6925 6930 6935 6940 6945 6950 6955 6960 6965 6970 6975 6980 6985 6990 6995 7000 7005 7010 7015 7020 7025 7030 7035 7040 7045 7050 7055 7060 7065 7070 7075 7080 7085 7090 7095 7100 7105 7110 7115 7120 7125 7130 7135 7140 7145 7150 7155 7160 7165 7170 7175 7180 7185 7190 7195 7200 7205 7210 7215 7220 7225 7230 7235 7240 7245 7250 7255 7260 7265 7270 7275 7280 7285 7290 7295 7300 7305 7310 7315 7320 7325 7330 7335 7340 7345 7350 7355 7360 7365 7370 7375 7380 7385 7390 7395 7400 7405 7410 7415 7420 7425 7430 7435 7440 7445 7450 7455 7460 7465 7470 7475 7480 7485 7490 7495 7500 7505 7510 7515 7520 7525 7530 7535 7540 7545 7550 7555 7560 7565 7570 7575 7580 7585 7590 7595 7600 7605 7610 7615 7620 7625 7630 7635 7640 7645 7650 7655 7660 7665 7670 7675 7680 7685 7690 7695 7700 7705 7710 7715 7720 7725 7730 7735 7740 7745 7750 7755 7760 7765 7770 7775 7780 7785 7790 7795 7800 7805 7810 7815 7820 7825 7830 7835 7840 7845 7850 7855 7860 7865 7870 7875 7880 7885 7890 7895 7900 7905 7910 7915 7920 7925 7930 7935 7940 7945 7950 7955 7960 7965 7970 7975 7980 7985 7990 7995 8000 8005 8010 8015 8020 8025 8030 8035 8040 8045 8050 8055 8060 8065 8070 8075 8080 8085 8090 8095 8100 8105 8110 8115 8120 8125 8130 8135 8140 8145 8150 8155 8160 8165 8170 8175 8180 8185 8190 8195 8200 8205 8210 8215 8220 8225 8230 8235 8240 8245 8250 8255 8260 8265 8270 8275 8280 8285 8290 8295 8300 8305 8310 8315 8320 8325 8330 8335 8340 8345 8350 8355 8360 8365 8370 8375 8380 8385 8390 8395 8400 8405 8410 8415 8420 8425 8430 8435 8440 8445 8450 8455 8460 8465 8470 8475 8480 8485 8490 8495 8500 8505 8510 8515 8520 8525 8530 8535 8540 8545 8550 8555 8560 8565 8570 8575 8580 8585 8590 8595 8600 8605 8610 8615 8620 8625 8630 8635 8640 8645 8650 8655 8660 8665 8670 8675 8680 8685 8690 8695 8700 8705 8710 8715 8720 8725 8730 8735 8740 8745 8750 8755 8760 8765 8770 8775 8780 8785 8790 8795 8800 8805 8810 8815 8820 8825 8830 8835 8840 8845 8850 8855 8860 8865 8870 8875 8880 8885 8890 8895 8900 8905 8910 8915 8920 8925 8930 8935 8940 8945 8950 8955 8960 8965 8970 8975 8980 8985 8990 8995 9000 9005 9010 9015 9020 9025 9030 9035 9040 9045 9050 9055 9060 9065 9070 9075 9080 9085 9090 9095 9100 9105 9110 9115 9120 9125 9130 9135 9140 9145 9150 9155 9160 9165 9170 9175 9180 9185 9190 9195 9200 9205 9210 9215 9220 9225 9230 9235 9240 9245 9250 9255 9260 9265 9270 9275 9280 9285 9290 9295 9300 9305 9310 9315 9320 9325 9330 9335 9340 9345 9350 9355 9360 9365 9370 9375 9380 9385 9390 9395 9400 9405 9410 9415 9420 9425 9430 9435 9440 9445 9450 9455 9460 9465 9470 9475 9480 9485 9490 9495 9500 9505 9510 9515 9520 9525 9530 9535 9540 9545 9550 9555 9560 9565 9570 9575 9580 9585 9590 9595 9600 9605 9610 9615 9620 9625 9630 9635 9640 9645 9650 9655 9660 9665 9670 9675 9680

**15**

2. The fuel composition according to claim **1** wherein the pour point of the fuel is about -40° C. to about -80° C., for use in a jet, rocket, or gas turbines.

3. The fuel composition according to claim **1** wherein the flash point of the fuel is about 38° C. to about 145° C.

4. The fuel composition according to claim **1** wherein the density is about 0.700 g/mL to about 0.900 g/mL.

5. The fuel composition according to claim **1** wherein the sum of carbons in the combined L moiety, R', and R" is from C<sub>5-14</sub>.

6. The fuel composition according to claim **1** wherein the A moiety is located on the alpha- or beta-carbon to the terminal carbon of the L moiety.

7. The fuel composition according to claim **1** which is essentially free of polycyclic aromatic substituents and essentially free of unreacted benzene.

15

**16**

8. The fuel composition according to claim **1** wherein the fuel composition is a jet fuel having a minimum smoke point of at least 20 mm.

9. The fuel composition according to claim **1** wherein the fuel composition is a diesel fuel having a cetane index of at least 40.

10. The fuel composition according to claim **5** wherein R' and R" are hydrogen and the A moiety is benzene.

11. The fuel composition according to claim **5** wherein R' is methyl and R" is hydrogen or methyl, and the A moiety is benzene.

12. The fuel composition according to claim **1** wherein the pour point of the fuel is about -20° C. to about -80° C., for use in diesel engines.

\* \* \* \* \*